

## UNITED STATES PATENT OFFICE.

ERNST AUGUST LAGE, OF HAMBURG, GERMANY.

## PROCESS FOR PRODUCING COLORED PHOTOGRAPHS (POSITIVE PRINTS ON PAPER OR THE LIKE).

No Drawing. Application filed July 25, 1921, Serial No. 487,527, and in Germany July 30, 1920.

This invention relates to a process for producing color prints on paper in non-fading colors by treating a silver black print from the part negative for the yellow print in a series of independent successive steps for developing the colors in the print to produce a final colored image similar to the object in nature.

The process includes the treatment of the print in a bleaching bath, a ferricyanid process to produce the blue portion of the image and a bichromate process for the red portion of the image, the last mentioned treatment developing the yellow portion of the image with the red, and a final fixing step which results in the production of the colored print.

The bichromate bath required for producing the bichromate yellow image is preferably utilized for exercising a simultaneous sensitizing action on the bichromate image.

The new process is carried out as follows:

An ordinary black silver print on gas light paper or the like is produced from the negative which is used for the yellow print. The silver black print is fixed and washed, and after fixing and washing, is introduced into a bleaching bath, the composition of which is substantially as follows:

Cubic centimeters.

|                                     |    |
|-------------------------------------|----|
| 10% lead nitrate                    | 15 |
| 10% potassium ferricyanide solution | 10 |
| 10% nitric acid solution            | 1  |
| Distilled water                     | 75 |

After the bleaching is completed, which changes the silver image of the print into a fading image, the print is thoroughly washed until the image no longer looks yellowish, and then dried. After the drying of the print, the print is moistened in subdued light by means of a cotton wool pad, with a solution consisting of:—distilled water, 60 cbc. cm.; ferric ammonium citrate, 7 gr.; potassium ferricyanide, 4 gr.

The paper thus coated and dried is now printed under the partial negative intended for the blue print, until the image becomes clearly visible. The printing with a normal

negative and in good daylight, takes 5 to 10 minutes. In any case it must be continued until all details of the image can be clearly seen, and the shadows begin to become gray. The blue print is thereupon rinsed in water until the lights appear clear, and the water dripping off from the print is no longer yellowish. After superficial drying, this print is uniformly coated with a 3% solution of potassium bichromate. After the drying, the print which is so far ready, is placed under the partial negative for red printing, and the printing is continued until the image becomes just visible in the brightest portions. The print is then rinsed, again, until the water running off is no longer yellowish, and placed on a flat support and properly dried. By completing the part negative for the red print on the paper rendered sensitive with the solution of potassium bichromate, the gelatine of the gas light paper is more or less tanned according to the influence of the light. By soaking in water a weak relief is then formed. Now, when the picture is rolled or dotted with red fat color, such color adheres only to those places which have been exposed to the light, and the result is the red part picture. After the bleached silver picture with the solution of potassium bichromate has been rendered sensitive to the light for the red part picture, the bleached silver picture is at the same time changed into a picture in oil. After a short fixing in sodium thiosulfate and subsequent rinsing and drying, the color image is ready.

It is especially important in the present process to keep the yellow partial image in invisible state until the blue and the red partial images have been printed.

Another advantage is that the bichromate solution spread on the print for the purpose of obtaining the red partial image, simultaneously develops the yellow partial image.

What I claim is:

A process producing colored photographic prints, consisting in subjecting a black silver print made from the yellow printing negative to a bleaching bath including lead ni-

trate, potassium ferricyanide, and nitric acid, resensitizing the print with a solution containing potassium ferricyanide and ferric ammonium citrate and printing from the 5 blue printing negative, washing and then resensitizing the print with a solution of potassium bichromate, printing from the

red printing print, applying red color for adherence to those parts of the negative which have been exposed to the light, and 10 fixing the sodium thiosulfate.

In testimony whereof I affix my signature.

ERNST AUGUST LAGE.